

Aug. 8, 1933.

P. J. MASSEY

1,921,368

PROCESS OF COATING PAPER

Filed May 29, 1930

2 Sheets-Sheet 1



Fig. 1.



Inventor:  
Peter J. Massey  
By Frank L. Billings  
Atty:

Aug. 8, 1933.

P. J. MASSEY

1,921,368

PROCESS OF COATING PAPER

Filed May 29, 1930

2 Sheets-Sheet 2



*Inventor:  
Peter J. Massey  
By Frank L. Bellman  
Atty.*

## UNITED STATES PATENT OFFICE

1,921,368

## PROCESS OF COATING PAPER

Peter J. Massey, River Forest, Ill.

Application May 29, 1930. Serial No. 457,110

11 Claims. (Cl. 91—68)

This invention relates to a method of coating paper with a suitable coating substance to produce thereon a coated surface having desirable characteristics for printing, and refers more particularly to the coating of paper as it passes from a portion of the driers of a paper machine, as a step in a continuous process of manufacture of coated paper.

This application constitutes a continuation in part of my earlier application, Serial No. 450,614, filed May 8, 1930.

The utility, objects and advantages of the invention will be apparent from the accompanying drawings and following detail description.

In the drawings, Fig. 1 is a diagrammatic side elevational view illustrating a portion of the apparatus suitable for carrying out my invention.

Fig. 1a is a diagrammatic elevational view of the remaining portion of such apparatus.

Referring in detail to the drawings, 1 indicates a pair of smoothing rolls interposed between a paper machine (not shown), which may comprise usual beating units, felting units, press rolls and the like, and a drying unit indicated generally at 3. The drying unit 3 may take the form of a conventional multi-tier drier having a plurality of upper drying rolls 4 disposed above a lower tier of drying rolls 5 staggered in a vertical plane from the upper rolls. Guide rolls 6 may be interposed between each of the rolls 4 comprising the upper tier of driers and are adapted to guide a continuous dry felt 7 which may be adapted to pass in turn over the upper surface of the drying rolls 4 and around the lower surface of the guide roll 6. The felt 7 may take the form of an endless unit, and upon passing over the upper series of drying and guide rolls 4 and 6, respectively, may return over a suitable arrangement of guide rolls 8, over tightening unit 9, and if desired may pass around a plurality of pony driers 10 and thence back to the wet end of drying unit 3.

A similar felt 7' may pass around the lower surfaces of each of the driers 5 and over the upper surfaces of guide rolls 6' suitably interposed between each of the driers 5. Felt 7' may return over guide rolls 8', over tightening unit 9', and if desired, over a plurality of pony driers 10' and back to the wet end of drying unit 3. The web 2 upon passing from smoothing unit 1 may be carried over the lower surface of the initial drying roll 5 of the lower tier, and thence may pass over the upper surface of the initial drying roll 4 of the upper tier and so on through the entire span of driers.

The web 2 upon leaving drying unit 3 may pass

to coating unit 11 wherein a suitable coating material may be applied to the continuously moving web 2 to produce a paper having a coated surface suitable for purposes of printing.

The coating unit 11 may comprise a fountain 60 or trough 12 adapted to contain a solution or suspension of coating material 13. The coating material 13 may be introduced to the container or fountain 12 through line 14, controlled by valve 15. The material 13 may be maintained in fountain 12 under superatmospheric, or, if desired, may be maintained at atmospheric pressure and may be transferred therefrom by gravity.

The material 13 may comprise a solution or suspension of suitable coating substances such as, for example, size, glue, gelatin, casein, starch, clay, calcium sulphate, resin, oils and/or varnishes carried and/or dissolved in a vehicle and/or diluent of water or oil. The proportion of liquid to soluble material may range in the approximate vicinity of 50%, more or less. It is to be understood, of course, that the hereinbefore mentioned examples and proportions are given merely for purposes of example and are not intended to serve in any way as a limitation upon my invention, since any of the well known materials for coating paper may be used and the exact proportions of solvents and/or vehicles to the binders and coating substances proper may be determined by the quality or character of coating to be produced and type of paper being coated.

A roll 16 may be journaled in such a manner as to rotate adjacent fountain 12 and may be adapted to contact the material 13 and thus have deposited a film of said material on its surface. The thickness of the film may be determined by proper regulation of a conventional doctor blade 17 operatively associated with the fountain and roll 16. Roll 16 may be constructed of metal or some like material.

A roll 18 may be journaled at one end of a swinging arm 19, the other end of which may be pivoted at 20. The surface of roll 18 may be constructed of rubber, or rubber composition, or some other material having relatively pliable properties. Arm 19 may be operatively connected and synchronized with the remaining elements of the apparatus to be hereinafter described in such a manner that at one period of operation roll 18 contacts roll 16, which action transfers a portion of the film on the surface of roll 16 to the surface of roll 18. At a subsequent period of the cycle roll 18 is swung into contact with the surface of a vibrating distributing drum 21, thereby transmitting its surface film to the surface of drum 21.

Said drum may be constructed of metal or other like material, the entire roll being adapted to vibrate or oscillate longitudinally, thereby tending to obtain a longitudinal distribution of said film upon its surface.

A rubber or compositioned-surface transfer roll 22 may contact roll 21 and hence transfer the film from roll 21 to its own surface. Transfer roll 22 may in turn contact vibrating distributing drum 23, which may, if desired, be constructed to vibrate or oscillate longitudinally, thereby further tending to establish a uniformly distributed film upon its surface. The drum 23 may be constructed of a material similar to that comprising drum 21.

A pair of transversely oscillating distributing drums 24 and 25 may be rotatably mounted adjacent drum 23 and may have their respective surfaces subjected to the film upon drum 23 through the agency of the pliable surfaced rolls 26 and 27, respectively. In this manner an extremely well worked film of coating material 13 may be established upon the surfaces of rolls 24 and 25, respectively.

By means of a plurality of pliable rolls 28 the film upon the surfaces of drums 24 and 25 may be transferred to the surface of coating roll 29. The surface 30 of roll 29 may be constructed of a relatively pliable material, such as rubber or rubber composition.

The coating roll 29 may comprise a portion of the coating unit proper which may consist of a base 31 upon which may be mounted upstanding guides 32. The lower coating roll 29', similar in construction to roll 29, may be mounted between the lower portion of guides 32 as at 33. The roll 29 may be mounted between guides 32 immediately above roll 29', the respective surfaces thereof being normally in contact. The contacting pressure of roll 29 upon roll 29' may be varied by the obvious manipulation of the system of linkages shown generally at 34.

It is to be understood, of course, that the various instrumentalities described in connection with coating unit 11 merely constitute one arrangement with which my invention may be carried out. Many other possible arrangements will suggest themselves to anyone skilled in the art, and I wish it to be understood that the invention is not in any way limited to the particular arrangement shown, which happens merely to be a form chosen to illustrate the invention.

Web 2 upon passing from drying unit 3 is carried forwardly between coating rolls 29 and 29' wherein a uniformly distributed film of coating material from the surfaces of said rolls is simultaneously transferred and compacted upon both surfaces of web 2. The web may then pass over a suitable guide roll 35 to an auxiliary drying unit 36, which may comprise conventional upper and lower drying rolls 4 and 5, respectively. Inasmuch as coating material 13 after passing over the series of transfer rolls described in connection with the coating unit loses a large proportion of its liquid content, principally by evaporation, the web 2 upon issuing from said coating unit needs a relatively short subsequent drying period, and hence the number of drying rolls 4 and 5 comprising unit 36 may be reduced to a minimum, and such auxiliary felt drying equipment as the pony driers 10 and 10' may be eliminated if desired. If desired, a drier felt 7 may be used in the final drying unit 36, or the felt may be entirely eliminated, or the first two or three rolls 4 and 5 of the unit 36 may be run

bare and a drier felt used upon the remainder of the rolls.

The web 2 upon issuing from drying unit 36 may pass to a stack of calender rolls 37 where-in the paper may be properly finished. Or, if desired, said web may be passed through both calender unit 37 and an additional calender unit 38. Upon issuing from the final calender stack 38 the paper may be reeled in any suitable manner (not shown). It is to be understood, of course, that any type calender or calenders may be utilized.

In passing through the coating unit 11 the coating material may be applied to one or both the rolls 29 and 29' and from the latter transferred to one or both surfaces of the web 2 in a uniform smooth film. Due to the efficient action of the various rolls constituting the coating unit 11 a solution or suspension of coating material may be used having a relatively low liquid content. As a result, due to the evaporation which takes place during the progress of the coating material through the rolls, the coating material applied to the web is in a relatively concentrated condition. Hence, the period of subsequent drying is reduced to a minimum and the coating material upon the surface, or surfaces, of the web needs no further working.

By suitably manipulating the doctor blade 17 and controlling the pressure of roll 29 upon roll 29' coatings may be applied to the web ranging in dry weight from approximately .05 to 5 pounds per one hundred square inches of paper, more or less.

As can be readily seen, the system of rolls appurtenant to coating roll 29' and designated by primed reference numerals is similar in all respects to the series described in connection with roll 29 and needs no further elaboration.

By properly controlling the feed of coating material from the troughs 12 and 12' to rolls 16 and 16', respectively, and by suitably gauging the contacting pressure of the coating rolls 29 and 29', a smooth film of uniform thickness of pre-worked coating material may be compacted upon said paper at any of the various speeds at which the paper machine proper may operate or, more strictly speaking, at any speed at which the web 2 may travel, it being possible to properly coat a web of paper moving at a speed of twelve hundred feet per minute, or higher, as uniformly and as well as a web moving appreciably slower.

By the term "worked" and/or "pre-worked" as used in the specification and claims is meant the step of reducing the coating material to the proper consistency for application to the web, as well as the step of progressively more uniformly distributing the film of material as the same is passed from roll to roll in the coating unit so that no further smoothing, scraping or brushing is necessary to produce a completely finished coated paper.

In utilizing my invention, as a step in a continuous process of manufacture of coated paper, the web after being properly felted and pressed, may be passed to a plurality of drying rolls, wherein the web is preferably thoroughly dried before passing to the coating unit. It is to be understood, of course, that the number of drying rolls immediately preceding the coating unit may be less than that sufficient to thoroughly dry the web, since the moisture content of the coating material when applied to the web is comparatively small and is not sufficient to detrimentally affect the paper in passing through the coating

unit. A relatively small number of drying rolls and a comparatively short drying period may follow the coating step, and what virtually occurs, is that the final driers of the paper machine are 5 divided into two sections and the coating unit interposed therebetween.

It is apparent that herein is provided a method of efficiently continuously applying a coating to a web of paper as the same passes through the 10 driers of a paper machine; a coating process which may accommodate itself to any of the various speeds now used in the manufacture of paper. A paper making machine when utilizing my invention presents not merely a machine and method 15 of making paper, but broadly comprises a machine and method for making coated paper.

By the use of the term "coated paper suitable for printing purposes" I intend to define the application of a coating substance to the paper of 20 a character conditioning the paper for printing thereon.

I claim as my invention:

1. A continuous progressive method of producing a uniformly coated fibrous sheet suitable for 25 printing purposes, which comprises the following steps: forming a continuous wet fibrous web, drying said web under elevated temperature, bringing said web into contact with moving surfaces carrying a uniformly distributed film of coating 30 material, simultaneously transferring said material as a pre-worked smooth finished coating to opposed sides of the web under pressure and drying said coated web, said pre-worked film being of relatively concentrated condition whereby it 35 will not detrimentally affect the fibrous web.

2. A continuous progressive method of producing a uniformly coated fibrous sheet suitable for 40 printing purposes, which comprises the following steps: forming a continuous wet fibrous web, drying said web under elevated temperature, bringing said web into contact with a moving surface carrying a uniformly distributed film of coating material previously transferred to said moving surface through a plurality of contacting moving 45 surfaces whereby the film is pre-worked and substantially dehydrated, transferring said material as a continuous finished coating to said web under pressure and drying said coated web, the concentrated condition of the pre-worked film being 50 such as not to detrimentally affect the web.

3. A continuous progressive method of producing a uniformly coated fibrous sheet suitable for 55 printing purposes, which comprises the following steps: forming a continuous wet fibrous web, drying said web under elevated temperature, treating a coating mixture, comprising a coating substance and a carrier, to eliminate a sufficient portion of the carrier to render the mixture suitable 60 for coating the fibrous web without detrimentally affecting the web, while simultaneously reducing the mixture to a desirable physical condition to smoothly coat the web thereafter coating the web with said reduced mixture and subsequently and without further working of the coating drying the 65 coated web.

4. A continuous progressive method of producing a uniformly coated fibrous sheet suitable for 70 printing purposes, which comprises the following steps: forming a continuous wet fibrous web, drying said web under elevated temperature, depositing a mixture comprising coating material and a liquid carrier on a moving surface, the viscosity of said mixture being below that desired for coating, transferring said mixture to a second 75 moving surface, working said mixture to cause it

to spread and form a uniform film on said second moving surface while simultaneously increasing the viscosity of the mixture, continuing such treatment until the mixture has reached the desired viscosity and is in the form of a uniform film having insufficient water to streak and detrimentally affect the web, then transferring said uniform film of desired viscosity to the fibrous web, simultaneously compacting the same thereon in the form of a finished coating and subsequently 80 drying said coated web.

5. A continuous progressive method of producing a uniformly coated fibrous sheet suitable for printing purposes, which comprises the following steps: forming a continuous wet fibrous web, drying said web under elevated temperature, passing said web between opposed rotating surfaces carrying preformed films of uniform thickness in which the coating material is uniformly distributed, transferring said preformed films simultaneously to opposite surfaces of said continuous 90 advancing web under the pressure of said opposed rotating surfaces as finished coatings the said pre-worked films being substantially dehydrated whereby there is insufficient water to detrimentally streak and affect the web.

6. The method of making coated paper suitable for printing purposes, which comprises the steps of treating the coating material to increase its viscosity by eliminating substantial quantities of 100 its liquid content and render it relatively plastic, advancing a web of fibrous material and transferring the treated material as a viscous and smooth film to the entire surface of the web under pressure whereby to obtain a final coated 105 product suitable for printing purposes.

7. The process of making coated paper for printing purposes, which comprises continuously advancing a web of paper, subjecting a coating mixture to mechanical working action to smooth 115 it and eliminate portions of the liquid contained therein and transferring said mixture as a mechanical pre-worked film to the advancing web under pressure, the liquid content of the film 120 being insufficient to detrimentally streak the web upon which it is transferred.

8. The process of making coated paper suitable for printing purposes, which comprises the steps of treating a coating mixture, comprises a coating 125 substance and a liquid carrier, to eliminate a sufficient portion of the carrier to render the mixture suitable for coating the paper without streaking the same while simultaneously reducing the mixture to a desirable physical condition to smoothly coat the paper, advancing a web of paper continuously and depositing said mixture upon the surface of the advancing web as a smooth finished coating therefor.

9. A continuous process of making coated paper 130 suitable for printing purposes, which comprises the following steps: depositing a mixture comprising coating material and a liquid carrier upon a moving surface, the viscosity of said mixture being below that desired for coating, transferring said mixture to a second moving surface, working said mixture to cause it to spread and form a uniform film on said second moving surface while simultaneously increasing the viscosity of the mixture, continuing such treatment until the mixture has reached a viscosity such as will not 135 detrimentally streak or affect the web and is in the form of a uniform film and then transferring said uniform film to a web of paper and simultaneously compacting the film thereon.

10. A continuous process of making coated 140

paper suitable for printing purposes, which comprises the steps of depositing a mixture including coating material, a liquid carrier upon a rotating surface, the viscosity of said mixture being below that desired for coating, transferring said mixture to a second rotating surface, working said mixture to cause it to spread and form a uniform film of said second rotating surface while simultaneously increasing the viscosity of the mixture, continuing such treatment until the mixture has reached the desired viscosity such as will not detrimentally affect the web, and is in the form of a uniform film, transferring said uniform film in its viscous state to a web of paper simultaneously compacting the same thereon, in the form of an unbroken, smooth coating, the viscous condition of the film minimizing the drying action required for the coated product.

20

95

25

100

30

105

35

110

40

115

45

120

50

125

55

130

60

135

65

140

70

145

75

150

11. The herein described process for making coated paper for printing purposes, the steps which comprise, advancing a web of fibrous material, subjecting a coating mixture to treatment during the advancing of the web for the purpose of eliminating substantial quantities of water content thereof, thereby mechanically working the mixture and in thereafter continuously transferring the viscous coating in the form of a pre-worked, smoothed, finished coating to the surface of the advancing web whereby to produce a final product with a smooth mechanically worked coating film thereon substantially free of streaks or other imperfections.

PETER J. MASSEY. 90

80

85

90

95

100

105

110

115

120

125

130

135

140

145

150